

Aug. 1, 1939.

F. PAVELKA

2,168,135

ELECTROLYTIC CONDENSER

Filed June 19, 1937



BY

FREDRICK PAVELKA  
E. H. HENDRICKSON  
ATTORNEY

## UNITED STATES PATENT OFFICE

2,168,135

## ELECTROLYTIC CONDENSER

Friedrich Pavelka, Klosterneuburg, near Vienna,  
Austria, assignor to Radiowerk E. Schrack Ak-  
tiengesellschaft, Vienna, Austria

Application June 19, 1937, Serial No. 149,266  
In Austria July 1, 1936

9 Claims. (Cl. 175—315)

My invention relates to electrolytic condensers, and more particularly to electrodes for such condensers.

One of the main advantages of electrolytic condensers is that, for the same voltage and load capacity, they have a much greater capacity for a given volume than do other types of condensers, such as paper condensers. Numerous attempts have been made to increase this advantage, for example by roughening the surface of the aluminum body serving as the anode, prior to its electrolytic oxidation by chemical etching, in order to greatly increase its surface area, i. e., to obtain a large etching factor.

15 The term "etching factor" as used herein is to be understood to mean a ratio which is generally determined indirectly by measuring the capacity obtained by using the same forming method with etched foil and with unetched foil; the ratio of 20 these capacities being approximately equal to the etching factor.

25 As the electrode bodies are generally in the form of foils, I shall refer to same hereinafter as foils for the purpose of simplicity; however this 25 is not intended to limit the bodies to aluminum foils, or to foils in general.

Attempts to obtain very high etching factors have been made by selecting particular chemical reagents for the etching process, or by selecting 30 definite concentrations or working temperatures. In such cases, however, it has been difficult or impossible to obtain very high etching factors which could be reproduced in mass production.

The main object of my invention is to obtain 35 electrodes for electrolytic condensers which have very high etching factors.

A further object of my invention is to provide electrodes of high etching factors which can be produced with uniformity in mass production.

40 Further objects of my invention will appear as the specification progresses.

As the result of extended metallographic research, I have found that there is a very close relationship between the etching factor obtained 45 and the grain size of the crystallites of the material of the foil, for instance of aluminum, and that the smaller the crystal grain size of the foil, the greater is the etching factor. While this etching factor is not inversely proportional to the grain size, it appears to be a logarithmic function thereof. In addition, however, the material of the foil should be such that the current loss, i. e., leakage current of the completed condenser, should be as low as possible.

In accordance with the invention I form such

electrodes of a material having a very small grain size, i. e., a very large number of crystals per unit surface area.

Very good results have been obtained by using aluminium in which the number of individual crystals at the active surface is of the order of and even more than  $10^9$  per sq. cm., which corresponds to a grain size of from 0.0001 to 0.001 mm. When making the electrodes of a condenser of such material, I obtain an etching factor up to 10 and exceeding 13.

By further decreasing the grain size of the aluminum foil of the anode I have found that etching factors up to 15 can be readily obtained. In forming such etched aluminum foils of for instance 0.2 millimeter in thickness in the usual electrolytic bath at a voltage of 650 volts, I secure a capacity up to and exceeding about 0.08 mfd. per sq. cm. of anode surface, for example 0.12 mfd. per sq. cm. of surface area. This increase in capacity is of great advantage, as in prior constructions a value of only about 0.1 mfd. was obtained. Thus with anodes having a crystal construction according to the invention, the surface may be only about half that required with 25 anodes having a maximum surface area.

To obtain the required small grain size, it is desirable to add very small quantities of admixtures to the aluminum. However I have found that greatly improved results are obtained by 30 using aluminum of a very high degree of purity, especially when the foil is relatively thick, for instance 0.2 mm. thick.

Electrolytic condensers using electrodes according to the invention and having identical capacity and identical voltage resistance, are considerably smaller than prior art condensers. For example, I can produce an electrolytic condenser which, for instance, at a working voltage of 500 volts and a capacity of 10 mfd. with the casing in a state of readiness for operation, occupies a space of only 15 cubic centimeters. Thus I obtain a specific capacity up to and above about 0.7 mfd. per cubic cm. and at lower operating voltages it is possible to obtain a correspondingly 45 higher specific capacity. In general, the invention permits of increasing the specific capacity of electrolytic condensers up to and above

350  
" mfd.

per cubic cm.;  $u$  designating the operating voltage. Thus the electrolytic condensers according to the invention permit a reduction in the size of various electrical apparatus, such as radio receiv-

5

15

20

25

30

35

40

45

50

55

ing sets, and their lower weight make them particularly useful in portable apparatus.

Preferably not only the anode, but in some cases also the cathode, should be made from the aluminum foil according to the invention, in order to give the latter a maximum surface area and thus to avoid the "connecting effect"; this expression being understood to mean the phenomenon of the gradual decrease in capacity brought about by a "sneaking" oxide formation on the cathode resulting from numerous connecting operations, which are always accompanied by a reversed passage of current.

In order that my invention may be clearly understood and readily carried into effect, I shall describe same in more detail with reference to the accompanying drawing, in which:

Figure 1 is a partly-sectionized side-view of a "dry" electrolytic condenser using an electrode according to the invention.

Fig. 2 is a microscopic view of a surface portion of the anode of Figure 1 and indicates the crystal structure; and

Fig. 3 is a microscopic cross-sectional view of the anode of Figure 1.

The dry electrolytic condenser shown in Figure 1 comprises a cup-shaped container 5 having its open end closed with a disc 4 of insulating material. Within container 5 is a condenser unit of the rolled type comprising two electrodes 1 and 2 of aluminum foil separated by a gauze spacer 3 carrying an electrolyte. The electrolyte comprises, for instance, a solution of ammonium borate and boric acid, and water and glycerine as the ionizing agent, and if desired also an inert substance; the electrolyte having a low fluidity, for instance a pasty consistency.

Electrodes 1 and 2 are provided with suitable terminals 6 and 7 respectively, extending through disc 4 in a liquid-tight manner.

In accordance with the invention, either one or both of the foils 1 and 2 is made from an aluminum foil of very small grain size, for instance smaller than 0.001 mm., and there are about 10<sup>6</sup> individual crystals per sq. cm. of active surface area (see Fig. 2).

The method of producing the material of the electrodes according to the invention is described and claimed in my copending U. S. patent application Ser. No. 149,265, filed June 19th, 1937; however I shall incorporate a description of the method in the present application in order to complete the disclosure.

The small grain size of the aluminum foil 1, which will be considered as the anode, may be obtained by means known for this purpose in metal working. For example, satisfactory results are obtained by rolling in a single rolling operation a comparatively thick aluminum foil, for instance 2 mm. thick, to a final thickness of about 0.2 mm. This 90% reduction in thickness produces the enormous increase in the number of crystal nuclei required by the invention. It is not essential that the rolling operation be effected in a single step, but it may be carried out in several steps, provided the usual heat treatment between the successive steps, which causes larger crystal individuals, is avoided. On the other hand, it is possible to use a heat treatment which is carried out in such manner that the internal stresses of the material are decreased without materially increasing the size of the crystals.

I have found that after rolling and prior to etching, it is preferable that the foils be sub-

jected to such a tempering operation, which may consist in transient heating. More particularly, after the foil has been reduced to its final thickness it may be heated to above about 270° C. On the other hand, the reduction in thickness may be effected in such a manner that crystal structure is shattered by the extreme deformation and the crystals are split up into very small particles, in which case recrystallization is prevented by avoiding prolonged subsequent or intermediate heat treatment.

To reduce the speed of recrystallization, the aluminum may have admixtures alloyed with it, care being taken that the admixtures be such that they do not increase the current of loss (leakage current) of the completed condenser. Such admixtures may be, for example, very small quantities, i. e., below 0.1%, of alumina, and also beryllium or tantalum, or the oxides of these elements.

I have found that greatly improved results are obtained when, instead of the admixture of slight quantities of impurities, the following procedure is followed.

As a result of systematic X-ray analysis research regarding the structure of aluminum in connection with the other chemical and physical constants of this material, I have found that aluminum having a very high degree of purity, i. e., a purity greater than 99.8%, and preferably greater than 99.98% has highly characteristic and surprising properties, which are very advantageous when the aluminum has crystal grains of the size of the present invention, i. e., smaller than 0.001 mm. and preferably of the order of magnitude of 0.0001 mm. A material having this grain structure may be recognized in radiographs by the absence of individual reflexes and the occurrence of permanent interferences; similar to those with colloidal solutions.

It is known that the greater the purity of base metals, such as aluminum, the better they can, as a rule, resist chemical attack by etching agents. This is probably because "local elements" are formed between the occluded impurities, the metal and the etching liquid, and these elements by electrolysis dissolve the metal, and the smaller amounts of impurities present, the slower this process proceeds.

I have found that in the case of aluminum the manner in which the chemical attack is effected is also influenced to a large extent by the grain size of the crystallites, and that by using aluminum of a particular purity, and of a particularly small grain structure of the material, a new product is obtained which is resistant to the etching, but which can be chemically etched to a great depth, thus increasing the etching factor.

For example, consider the case of an aluminum foil about 0.2 mm. thick and having a fine-grained crystal structure, i. e., a prevailing grain size about 0.0003 mm., and a degree of purity of about 99.99%. If this foil is subjected for about 16 hours at a temperature less than 20° C. and preferably between 10° and 15° C., to the action of concentrated commercial hydrochloric acid that may have 20% of water added to it, and it is subsequently washed and dried, the foil will have lost about 45% in weight, whereas no substantial decrease in thickness can be determined by a micrometer. On the other hand, if a commercial aluminum foil having a purity of about 99.7% were subjected to the same treatment, it would be completely dissolved in a few minutes.

If a drop of water is placed upon the silky shining surface of the etched foil made by the above process, it is greedily sucked up and forms a wet spot which soon becomes visible on the reverse side of the foil. This proves that the foil was "etched through" under the experimental conditions above specified, i. e., it is traversed by a large number of exceedingly fine pores which constitute a connection between the two surfaces, such as indicated in Fig. 3. These pores or hollows are of substantially the same size as the crystals.

In contradistinction to the unetched foil, which is absolutely opaque, it is observed upon intensively illuminating one surface of the etched foil, that there is on the opposite surface a diffused luminous glimmer which may obviously be accounted for by repeated reflection of light on the irregular walls of the minute pores formed in the foil.

That a spongy structure of great fineness, for example such as indicated in Fig. 3, is produced, is shown by the marked capillary action of such foils. For example, if a dry strip of the etched-through aluminum foil is placed in pure water at ordinary temperatures, the water rises by capillary action to a height of about 22 cms. After electrolytic oxidation of the surface of the foil, which may be effected in the well known manner, the height to which the water will rise is decreased, for example to 10 cms., by reason of the altered capillary constant of the material. The marked reduction in vapor pressure of the sucked-up liquid, which is closely related to the capillary action, is also remarkable.

The electrolytic oxidation can be carried out in a bath containing boric acid and ammonia, dissolved in distilled water, the latter being as free from chlorine as possible. The formation tension is slowly increased till it reaches the value of about 650 volts.

An aluminum foil suitable as a starting material for the etching process described above, may be obtained in the following manner: A sheet of extremely pure aluminum, for instance a purity of about 99.99%, having the usual crystal size, i. e., grain-size about 0.1 mm. and a thickness of about 2 mms. or even larger, is used as the starting material. This sheet is rolled in one or more steps to a final thickness of about 0.2 mm. For example, 2 rolling steps may be used with a 45% reduction in thickness for each step. During the rolling operations the usual grain-increasing intermediate heating operations, which are usually used between the rolling operations, are not used. As has been set forth above, this extreme decrease in thickness shatters the crystal individuals so that the required small-grain structure is set up. Although with aluminum having a lower degree of purity, such extreme deformation produces an extremely strong strain on the rolling tools because a product of great hardness is obtained, this is not true to the same extent with very pure aluminum which remains comparatively soft in spite of the extreme change in form. This is also of importance in connection with the treatment subsequent to the rolling process.

Particular care must, of course, be taken that the purity of the foil is not decreased during the process, for example by particles of the roller surface sticking to it.

After the final rolling operation the foil can be "tempered", i. e., subjected to a heat treatment which, however, as above stated, should

be so carried out that merely a relaxation but no increase in size of the crystals takes place. For this purpose the heat treatment should not be effected above about 270° C. and should preferably be so carried out as to insure that no differences in temperature are set up between the individual parts of the foil, i. e., by slowly heating the foil to the desired temperature.

The crystal grains produced in the foil by the above method are not arranged in a completely irregular manner, but form a fibrous structure similar, for example, to the fibrous structure of unfired drawn tungsten wire. The presence of this fibrous structure can be ascertained, particularly after the etching, by the fact that a drop of liquid dropped upon the etched foil does not flow out to form a circle but forms an ellipse whose major axis coincides with the rolling direction. This structure should be taken into account during the further working, i. e., during the folding, rolling, etc., of the foil.

After being rolled and tempered in the above manner, the foil has an oxide film which is harmful for many purposes. For example, etching of the above-described type can only be effected after removal of this oxide film, as otherwise even the concentrated hydrochloric acid would not attack the foil. It is characteristic of the chemical resistance of pure aluminum foil that the oxide film cannot be removed with a bath of lye, whereas this is directly possible in the case of commercial foils. It is therefore advisable that the oxide film be removed mechanically, for example by a rotary steel brush. This brushing operation should, however, be effected in a very cautious and delicate manner, not only to avoid introduction of impurities but also to prevent local increases in temperature and surface irregularities which would affect subsequent attack by etching acid.

The new material produced in the above manner is highly suitable for being used, according to the invention, as an electrode in electrolytic condensers whether the electrode is in the form of a foil, wires, profiled rods, tubes, etc.

Since it is possible for aluminum foil, according to the invention, to be etched through without otherwise losing its coherence, the total active surface which can be obtained—and thus the etching factor—is also dependent on the thickness of the initial material. The etching factor is therefore a function not only of the material used, but also of the shape of this material. Although the etching factor increases with the thickness of the foil, it does not increase linearly with the thickness but in a smaller degree so that there is a maximum foil thickness-dependent on the etching process, the grain size, and the degree of purity above which there is no appreciable increase in the etching factor.

The degree of purity of the material is particularly important in connection with the depth of etching, because with metal containing more than 0.2% of impurities, particularly heavy metals, the etching process proceeds in a different manner, i. e., the etching proceeds essentially parallel to the surface, and not in the perpendicular direction, and the etched pores are coarser and smoother. Although it would appear that the etching proceeds most rapidly along the grain surfaces, and that the new material because of its very fine structure assists the advance of the etching in the depth direction, this theory per se must be considered insufficient because the material would be split up during etching into a

powder. This, however, is not the case, because the individual grains of the spongy material produced during etching have relatively large metallic coherence. On the other hand, the pores are interconnected to form the spongy-like material.

The purer the material used, the more concentrated must be the etching liquid, for example hydrochloric acid, and the longer this liquid must act to produce the desired degree of etching. On the other hand, the optimum composition and acting time of the etching liquid is also dependent upon the thickness of the foil to be etched. In the case of excessive foil thicknesses, for example above 0.2 mm., the "etching through" is more difficult because, due to the prolonged acting time required, the portions of the foil nearer the surface are attacked to an excessively high extent. Furthermore, if after "etching through" the etching liquid is allowed to continue its action, the factor of the increase in surface is again decreased.

It is advisable that during the manufacture, samples be taken from time to time, for example after rolling, and the grain size tested by X-rays. Furthermore, the extent to which the grain size has advanced should be determined during the etching, since the etching time is dependent not only upon the initial degree of purity of the metal, but also upon the type of impurities present and upon the amount of reaction products in the etching liquid. For instance comparatively small quantities of aluminum chloride in the hydrochloric acid expedite the etching process.

While I have described my invention in connection with a foil electrode and a "dry" electrolytic condenser of the rolled type it is not limited to such, but is equally applicable to electrodes of other shapes and to electrolytic condensers of other types. Furthermore, the invention can be used in connection with either the anode or cathode or both. Therefore, I desire the appended claims to be construed as broadly as permissible in view of the prior art.

What I claim is—

1. An electrode for an electrolytic condenser comprising an etched body of aluminum containing less than 0.05% of impurities, the crystal grain size of the aluminum being less than 0.001 mm.

2. An electrode for an electrolytic condenser

comprising an etched body of aluminum containing less than 0.02% of impurities, the crystal grain-size of the aluminum being less than 0.001 mm.

3. An electrode for an electrolytic condenser comprising an etched body of aluminum containing less than 0.02% of impurities and having a crystal grain-size less than 0.001 mm., the surface of said electrode having a spongy structure with hollows about equal to the grain-size.

4. An electrode for an electrolytic condenser comprising a body of aluminum containing less than 0.02% of impurities and having a crystal grain-size less than 0.001 mm., said body being etched through and having throughout a spongy structure provided with hollows about equal to the grain-size.

5. An electrode for an electrolytic condenser comprising a body of aluminum containing less than 0.02% of impurities and having a crystal grain-size less than 0.001 mm., said body being etched through and having a spongy structure and a capillarity for pure water at 20° C. of at least 8 cms.

6. An electrode for an electrolytic condenser comprising an etched body of aluminum containing less than 0.02% of impurities and having a crystal grain-size less than 0.001 mm., the system of crystallites of said body having a fibrous structure.

7. An electrode for an electrolytic condenser comprising an etched body of aluminum containing less than 0.05% of impurities and having a crystal grain-size less than 0.001 mm., said body having an etching factor greater than 13.

8. An electrode for an electrolytic condenser comprising an etched body of aluminum containing less than 0.05% of impurities and having a crystal grain-size less than 0.001 mm., said body having an etching factor greater than 15.

9. An electrolytic condenser comprising an electrolyte and electrodes including an etched aluminum body containing less than 0.05% of impurities and having more than 10<sup>9</sup> crystal individuals per sq. cm. of active surface, and a dielectric film formed on the surface of said body at about 650 volts, said condenser having a capacity of about 0.08 mfd. per sq. cm. of the unetched surface of said body.

FRIEDRICH PAVELKA. 50